

## UNITED STATES PATENT OFFICE

GEORGE E. RICE, OF BROOKLYN, NEW YORK, ASSIGNOR, BY DIRECT AND MESNE ASSIGNMENTS, TO CONSERVATION CORPORATION OF AMERICA, A CORPORATION OF DELAWARE

## METHOD OF PRODUCING WOOD PULP

No Drawing.

Application filed January 24, 1924. Serial No. 688,350.

The present invention relates to the production of wood pulp or fibrovascular cellulose from woods and plants, for the manufacture of paper, fibre board, and the like, and 5 the fundamental object of the invention is to provide a novel process for treating the wood in a simple, practical and efficient manner, in order to remove the extraneous matter and obtain a high grade cellulose fibre of maximum 10 strength, which separates easily, and which will combine or mat perfectly in making paper or fibre board.

Another object is to provide such a method 15 of producing wood pulp, which is not only highly efficient for well known pulp woods, but which also enables a high grade wood pulp to be obtained from several classes of woods not suitable for wood pulp by prevailing processes, thereby making such additional woods available for high grade pulp 20 which have heretofore been difficult or impossible to bleach thoroughly. For example, the present process is suitable and efficient for such woods as Douglas fir, larch, hemlock, 25 Mississippi red gum, Maine spruce, Canadian spruce, Louisiana cypress, Oregon pine, pitch pine, soft maple, resin pine, Kentucky poplar, *Hura crepitans*, white oak, red oak and soft white pine, some of which, as known to 30 the trade, are considered unsuitable for the production of a high grade pulp.

A further object is the elimination of the treatment of the wood, as in prevailing processes, by reagents under pressure, such as in 35 digesters, and the elimination of incidental complicated apparatus and cumbersome handling and manipulation of the materials, and the present process enables the wood to be treated, for the extraction of foreign matter 40 therefrom, in open tanks under atmospheric pressure. The hazard of escaping fumes is thereby dispensed with, which is a menace to the workmen and others in the vicinity of pressure apparatus, especially when dangerous 45 reagents are used, such as halogens, which are destructive to life.

One phase of the process contemplates the treatment of the wood in its natural state, for the purpose of removing the extraneous matter therefrom, such as the starch, sugar, gum, 50

acid, oil, resin, albumin, tannin, etc., in order to prepare the wood for bleaching, without using dangerous reagents or pressure.

The other phase of the process resides in the bleaching of the treated wood in such a 55 way as to be improved and thoroughly efficient in connection with the first phase of treatment of the wood, in order to obtain a thoroughly bleached fibre of high grade.

In carrying out the process, the logs are 60 first prepared by removing the bark and small branches, and the wood, either the whole logs or sticks or blocks, are then boiled in a saccharine (sugar-like) solution, in order to extract the foreign matter, the term 65 "saccharine" being used herein with the adjective meaning to indicate a sugar or sugar-like solution. Such solution may vary according to the different grades of woods treated, and according to other circumstances. 70 For example, a typical solution comprises 1,200 pounds of water, 360 pounds of sugar (50% dextrose and 50% levulose) and 75 pounds of prepared dextrin, the sugar and dextrin providing the mixed carbohydrates. 75 These proportions may vary according to the different grades of woods treated, but the amount of sugar is substantially 25% of the amount of water, and the amount of dextrin is substantially 5% of the amount of water. 80 When it is desired that the finished product be insect and fungi proof, and to prevent rot, sodium fluoride is added to such solution amounting to substantially 2% of the total weight of the solution, or for the proportions given, 32 pounds of sodium fluoride. 85 The specific gravity of such solution at a temperature of about 60 degrees F. would be about 1.090, which will permit of the solution being thinned according to the density or 90 absorption characteristics of the wood to be treated. The average specific gravity of the solution, during the treatment, should be between 1.075 and 1.085, and only water is added for thinning the solution to the desired 95 specific gravity. There is also added to such solution  $\frac{1}{2}$  of 1% of soda ash (95%), based on the total weight of the solution, or approximately 2% of the amount of sugar or carbohydrate. The addition of sodium sul- 100

phite to the solution, in an amount substantially five percent of the solution, has been found to also materially assist in the deserialization of the wood and the bleaching thereof.

5 Such liquor or solution is heated in any suitable open tank, by means of steam coils or the like, to a temperature that may vary from 100 to 150 degrees F., and the wood is then immersed in the solution. The immersing of the wood can be accomplished in different ways, and the wood can be loaded on trucks, skids or other carriers for conveying the wood into and out of the tank without 10 individually handling the pieces of wood.

15 When the wood is immersed in the solution, the solution is heated to gradually raise the temperature to 212 degrees F., or the boiling point of water, and the boiling is continued until all extraneous matters are removed from the wood. During the boiling of the wood, scum and froth rise to the surface, and are skimmed off, and the skimmings are 20 preserved, and are used as fertilizer and other valuable by-products. When the wood has been boiled a sufficient length of time, ranging anywhere from a fraction of an hour to several hours, and no further scum rises to the surface of the liquor, then the solution 25 is permitted to cool down to not lower than approximately 170 degrees F. and wood is removed. The solution is at once ready for the next load of wood.

30 The wood is preferably dried before grinding, either naturally or artificially, artificial drying being used for rapid production. Any suitable steam-heated or equivalent dryer can be used.

35 The wood is then ground up, either dry or wet, but preferably dry, into small shreds or particles, and is then ready for bleaching.

40 The saccharine substance used may be a low grade syrup or molasses, either cane, beet or corn, or other form of sugar or invert. When 45 a mixed carbohydrate solution is used, dextrin is mixed with the sugar. The dextrin may be of corn, potato or other dextrinized starch. Black strap molasses and other low grades of molasses and syrup are used to advantage, being cheap forms of sugar, and 50 containing impurities which are beneficial in the treatment and bleaching of the wood. Such low grades of molasses and syrups contain sulphur dioxide, which is useful in further preparing the wood for bleaching. In 55 fact, the present process enables low grade molasses to be used, which is not suitable for human consumption, especially when such molasses contains over 350 parts per million 60 of sulphur dioxide, which is the limit permitted under Government requirements. Molasses and syrups containing sulphur dioxide in excess of such amount can be used to advantage in the present process, and when the 65 sulphur dioxide content of the molasses or

syrup is lower, it can be increased by the addition of sulphur dioxide, so that the saccharine solution contains a desired small percentage of the sulphur dioxide.

70 During the boiling of the wood in the saccharine solution, the solution enters the pores of the wood by osmotic action, and will dissolve the foreign matter in or expel it from the wood, such as starch, sugar, gum, acid, oil, albumin, tannin, and the like, and as the 75 boiling continues the deleterious or undesirable elements are thus extracted from the wood by the boiling solution, until finally, after the boiling has been continued a required length of time, the wood is near a condition of pure cellulose, containing only such small remaining portion of the solution as can be readily eliminated in the bleaching step. The sugar or saccharine solution has the ability, by osmotic action, to penetrate 80 the colloidal cell walls of the wood, with an efficiency that is not possible with water alone or with other substances previously suggested or used in the art. The osmotic action is of considerable benefit in penetrating the 85 cell walls, without using a closed tank, in order that the foreign matter may be dissolved, or discharged from the cells. During the boiling action, the lignin components of the wood are removed; portions of actual 90 incrusting matters are gelatinized and converted into colloidal condition; the starches and gummy matters are removed; and the saps and natural moisture are vaporized.

95 The extraneous matters are eliminated without discoloring the cellulose, and the treatment does not weaken the fibres as in prevailing processes, whereby the fibers have maximum strength. Some of the foreign matter rises to the surface of the solution as scum 100 and is skimmed off, and the balance leaves as vapor. The presence of the soda ash in the solution will, by a neutralizing action on the acid in the wood, form a sodium salt, the 105 nature of which depends on the particular acid in the wood, and in the reaction that takes place, carbon dioxide is liberated, which 110 helps or assists in expelling loosely or mechanically combined substances present in the wood.

115 The same treatment is used for plants which are of a woody or semi-woody nature, and which are available for the production of fibre pulp. The pulp produced from the wood or plant may not only be used for making paper, fibre and wall board, and the like, but may also be used for the production of pure cellulose to be used for the manufacture of fibre silk, gun powder, etc. The cellulose of the wood or plants being extremely inert 120 or non-reactive, resists the hydrolyzing action of alkalis and acids, and has no tendency to combine directly with the halogen elements (chlorine and bromine) so that the desired element of the wood (cellulose) re- 125 130

mains unaffected by the treatment to which the wood is subjected in the present process.

For some woods, black strap molasses and corresponding low grades of molasses and syrups can be used alone, with water, without the addition of dextrin. For example, three and one-half pounds of such low grade molasses or syrup is used with each gallon of water, and the sulphur dioxide content of the molasses or syrup makes such molasses or syrup especially suitable and advantageous for the present process, inasmuch as the sulphur dioxide or sulphite, during the boiling of the wood in the solution, is distributed throughout the wood in minute quantity, and, by the formation of sulphuric acid, will attack and remove foreign matter in the wood which may not be affected by the saccharine. The wood is therefore better prepared for the bleaching step.

The ground up treated wood is then bleached, preferably after the fibre has been dried, although the wet fibre can be bleached with success. The bleaching is done by means of the action of a sodium or calcium hypochlorite solution on the coloring material remaining in the wood. The action differentiates from prevailing bleaching processes, in so far as mechanical procedure is concerned, inasmuch as it is necessary to only have a slight mechanical agitation, and the bleaching is done at a temperature not exceeding 75 degrees F. The manufacture of the hypochlorite solution may be by any of the well known methods, but electrolytic hypochlorite is especially suitable, notably when a complete bleaching action is desired. The fibre is introduced into the solution of hypochlorite, and is allowed to remain therein from four to twelve hours, dependent on the type of wood that is being bleached. Only slight mechanical agitation is necessary, and the bleaching action will remove the last traces of coloring and foreign matters from the fibre, with the result of a perfectly bleached fibre or pure cellulose.

After the fibre is bleached, it is removed from the bleaching solution, and is then washed thoroughly in water, and dried. The cellulose thus produced can then be used at once for the production of paper, fibre board, gun powder, artificial silk, etc.

The sodium sulphite, when added to the saccharine solution, will also assist materially in the bleaching of the wood, in addition to deresinating the wood during the boiling thereof.

Having thus described the invention, what is claimed as new is:—

1. The process of producing wood pulp, consisting in boiling wood in water containing a substantial proportion of one or more carbohydrates, until no further scum rises to the surface, and then bleaching the wood.

2. The process of producing wood pulp,

consisting in boiling wood in water containing a substantial proportion of one or more carbohydrates and also containing sodium fluoride, soda ash and sodium sulphite, and then bleaching the wood.

3. The process of producing wood pulp, consisting in boiling wood in water containing a substantial proportion of one or more carbohydrates and also containing sodium fluoride, and then bleaching the wood.

4. The process of producing wood pulp, consisting in boiling wood in water containing a substantial proportion of one or more carbohydrates and also containing soda ash in an amount approximately 2% of the amount of carbohydrate, and then bleaching the wood.

5. The process of producing wood pulp, consisting in boiling wood in water containing a substantial proportion of one or more carbohydrates and also containing sodium sulphite, and then bleaching the wood.

6. The process of producing wood pulp, consisting in boiling wood in water containing a substantial proportion of sugar, until no further scum rises to the surface, and then bleaching the wood.

7. The process of producing wood pulp, consisting in boiling wood in water containing a substantial proportion of sugar and also containing sodium fluoride, soda ash and sodium sulphite, and then bleaching the wood.

8. The process of producing wood pulp, consisting in boiling wood in water containing a substantial proportion of sugar and also containing sodium fluoride, and then bleaching the wood.

9. The process of producing wood pulp, consisting in boiling wood in water containing a substantial proportion of sugar and also containing soda ash in an amount approximately 2% of the amount of sugar and then bleaching the wood.

10. The process of producing wood pulp, consisting in boiling wood in water containing a substantial proportion of sugar and also containing sodium sulphite, and then bleaching the wood.

In testimony whereof I hereunto affix my signature.

GEORGE E. RICE.

120

125

130